

## UNITED STATES PATENT OFFICE

HORATIO A. HELDER, OF CANTON, NORTH CAROLINA, ASSIGNOR TO THE CHAMPION FIBRE COMPANY, OF CANTON, NORTH CAROLINA, A CORPORATION OF OHIO

## BLEACHING FIBER PULP

No Drawing.

Application filed June 15, 1928. Serial No. 285,782.

This invention relates to a process of bleaching fiber pulp; more particularly, it is concerned with an improvement in a process of bleaching wood pulp.

5 It heretofore has been known in the art that, in the process of bleaching fiber pulp,—for example, wood pulp,—the speed of bleaching, and removal of the products of the bleaching treatment by washing with 10 water, can be greatly facilitated by slightly acidifying the fiber prior to the conclusion of the bleaching operation. It has been known, also, that the rate and character of the bleaching treatment are determined to 15 some extent by the suitable adjustment and maintenance of the hydrogen ion concentration of the water suspension of the fiber pulp during the treatment: for example, too low a hydrogen ion concentration may result in 20 an excessive increase in the time required to complete the bleaching action. A favorable degree of acidity is that represented by pH values between 4.0 and 3.0.

I have found that the bleaching of fiber 25 pulp by means of commonly used bleaching agents, such as, for example, a solution of bleaching powder, and the removal of the products thereof, may be facilitated by the addition to the fiber pulp of an aqueous liquid 30 obtained as condensate from the evaporation concentration of dilute tannin extract, which aqueous liquid is known in the art as "sweet water".

In the extraction of tannic acid and other 35 tannins from wood and/or wood bark,—for example, from the bark or/and woody parts of the American chestnut tree,—by means of hot water, there are extracted at the same time other water-soluble organic compounds which are,—with relation to tannic acid,—relatively volatile. The resulting aqueous extract is relatively dilute and requires concentration in order to obtain a commercially useful extract of high tannin 45 content. In general practice, the concentration is effected by evaporation,—usually, by vacuum distillation by means of multiple effect evaporators. During the concentration operation there are volatilized water and at 50 least a part of the said volatile, water-soluble,

organic compounds extracted from the wood or bark. Upon condensation, there is obtained the aqueous acidic condensate,—known as "sweet water",—the use of which in the bleaching of fiber pulp forms the basis of 55 the present invention. This aqueous acidic condensate heretofore has been a waste material causing difficulty in its disposal.

I have found that the aqueous condensates obtained from the evaporation concentration 60 of dilute tannin extracts have an acid reaction equivalent in acidity to approximately 0.006 normal, and may have a pH value of 3.8,—i. e., within the range 4.0 to 3.0 hereinbefore described as representing favorable 65 acidities of the wash waters and/or pulp.

I have found that the addition of the above-described aqueous acidic liquid obtained as condensate from the evaporation concentration of tannin extract to the unbleached pulp 70 or to the pulp undergoing bleaching treatment results in a more rapid bleaching and in an economy of bleach.

The substitution thereof for a dilute acid 75 in the known bleaching processes effects an improvement in the quality of the resulting bleached pulp and an economy of bleach, and as well opens up a field of usefulness for this hitherto-considered waste material.

The "sweet water" may be added to the 80 pulp in such manner as to displace the residual water in a pulp which has been thickened to a consistency of about 8% or more; or, it may be added at the conclusion of the bleaching treatment and prior to washing; 85 or, in order that the "sweet water" may have ample opportunity to penetrate the pulp fibers, it may be added to the partially bleached pulp in a single stage or in successive stages during the period of bleaching. 90 I have discovered that, by the use of this "sweet water", the bleach residues are readily removed and that a pulp of superior whiteness is obtained, while effecting an economy in the consumption of bleach and of heat. 95

It is to be understood that the invention embraces the use of the hereinbefore described "sweet water" as a substitute, wholly or in part, for the dilute aqueous acid solutions previously employed, and also that the 100

acidity of the "sweet water" may, if desired, be adjusted as on the one hand by dilution or on the other hand by addition thereto of a regulated small amount of acid.

5 I claim:

1. In processes of bleaching fiber pulp, the step which consists in the addition to the pulp at any stage prior to the removal of bleach residues therefrom by water washing of an aqueous condensate from the evaporation concentration of an aqueous tannin extract.
- 10 2. In processes of bleaching fiber pulp, the step which consists in the addition to the pulp at any stage prior to the removal of bleach residues therefrom by water washing of an aqueous condensate from the evaporation concentration of an aqueous tannin extract, said condensate having an acidity falling within the range of pH values of 4.0 to 3.0.
- 15 3. In processes of bleaching fiber pulp, the step which consists in the addition to the pulp prior to the bleaching treatment of an aqueous condensate from the evaporation concentration of an aqueous tannin extract.
- 20 4. In processes of bleaching fiber pulp, the step which consists in the addition to the pulp prior to the bleaching treatment of an aqueous condensate from the evaporation concentration of an aqueous tannin extract, said condensate having an acidity falling within the range of pH values of 4.0 to 3.0.

25 In testimony whereof, I affix my signature.

35 HORATIO A. HELDER.

40

45

50

55

60

65